

1

2,990,303

## CONDITIONING TREATMENT FOR COOLING SYSTEMS AFTER ACID CLEANING

Charles F. Pickett, Bel Air, and Myer Rosenfeld, Baltimore, Md., assignors to the United States of America as represented by the Secretary of the Army

No Drawing. Filed Jan. 7, 1960, Ser. No. 1,140

9 Claims. (Cl. 134—22)

(Granted under Title 35, U.S. Code (1952), sec. 266)

The invention described herein may be manufactured by or used for the Government for governmental purposes without the payment to us of any royalty thereon.

This invention relates to a process and composition for prolonging the use life of internal combustion engine cooling systems and more particularly concerns a process and composition for conditioning such cooling systems subsequent to treatment with acid cleaning compositions.

Various acid, cooling system cleaners are known to the art. Of particular interest in this respect is the highly effective acid cleaner disclosed in U.S. Patent No. 2,631,950. Normally, after treatment with such acid cleaners, an ordinary flushing operation is employed to completely remove the acid and loosened soil. Previously, it was thought that such ordinary flushing was sufficient to accomplish this purpose. However, it has been found that after a few months use of cooling systems that have been acid cleaned and flushed in the usual manner there is a noticeable increase in the chloride content of the coolant. For example, a coolant having an initial chloride content of 6 parts per million in a month was found to have a chloride content of 200 parts per million. This build up of chloride content is due to the presence of soil which was loosened during the acid cleaning process but was not removed by conventional flushing processes. This loosened soil gradually enters the coolant, carrying with it entrapped chlorides. Although it has long been recognized that a very thorough flushing is needed subsequent to the acid cleaning of cooling systems, it was not previously realized that such flushing is ineffectual in removing soils which have been loosened but not actually removed from the surfaces of the cooling system which has been acid cleaned.

Accordingly, an objective of this invention is to provide means for conditioning acid cleaned cooling systems.

A further object of the invention is to provide a method for the removal of residues loosened by acid cleaners but not removed without the use of a flushing machine.

A further object of the invention is to provide a process and composition that is capable of deactivating the surfaces of internal combustion engine cooling systems.

Briefly, the conditioning treatment of this invention involves two separate phases or steps. The first phase consists of circulating through the system an alkali metal silicate solution. The second phase consists of circulating through the system an alkaline rinse solution. The alkaline solution comprises a mixture of an alkali metal phosphate and an alkali metal borate. The alkaline rinse solution may optionally contain sodium carbonate. The

two phases must be performed separately. Incorporating the silicate treatment with the alkaline cleaning step offers no advantage over no silicate at all. The one must necessarily follow the other to obtain the desired result. Therefore, the silicate solution must be drained from the system before the alkaline rinse is introduced.

After a water cooling system has been acid cleaned, with perhaps, the acid cleaners of the type disclosed in U.S. Patent 2,631,950 and the system thoroughly flushed with water the process of this invention is then applied. Sufficient alkali metal silicate solution is added to the system to obtain a concentration of silicate of from about 0.5 to 4.0 percent by volume. The system is then brought to a temperature of from about 160°—180° F. for approximately fifteen minutes and is then drained. If desired, this latter period may extend anywhere from five minutes to four hours. The system is refilled with fresh water, leaving some space for the alkaline rinse solids that are to be added or, if preferred, the alkaline solids may be added in the fresh water. The alkaline solids comprise a mixture of an alkali metal phosphate or polyphosphate and an alkali metal tetraborate. The preferred alkali metal phosphate is trisodium phosphate and the preferred alkali metal tetraborate is sodium tetraborate. The alkali phosphate is present within a concentration of from about 0.5 to 4.0 percent by weight. The alkali tetraborate is present within a concentration of from about 0.5 to 3.0 percent by weight. Sodium carbonate may optionally be included in the alkaline rinse solution in concentrations up to about 1.0 percent by weight. This system is brought to a temperature of from about 160°—180° F. for approximately five minutes to four hours.

It has been discovered that the important consideration in conditioning the cooling systems is not so much to obtain superior inhibitory action, as it is to strike a balance between deactivation of the surface and thoroughness of elimination of residue loosened by the acid cleaning treatment but not removed by the subsequent water flush. This balance concerning deactivation of the surface and elimination of residue is attained following the two-step process disclosed herein. The experimental evidence shows that the multiple components of the second step, the alkali metal phosphate and tetraborate, act together synergistically to provide for better surface deactivation than is obtained when the components are used individually. By X-ray diffraction analysis of the adhering deposits in the cooling system it was determined that there was a fundamental difference between the silicated treated systems and those not so treated. The two-step conditioning treatment is known to produce a very effective coating on the metal surface that deactivates said surface. This new conditioning process can extend the use life of the cooling system over four times that realized with the current conditioning methods.

The following are working examples given for the purpose of specifically illustrating how the process may be performed.

Various illustrations of concentration coming within the scope of the invention are the following:

|                                                                                                                                                           | 1   | 2    | 3    | 4   | 5   | 6   | 7    | 8   | 9   | 10  | 11  | 12   |
|-----------------------------------------------------------------------------------------------------------------------------------------------------------|-----|------|------|-----|-----|-----|------|-----|-----|-----|-----|------|
| (a) Sodium silicate solution, 40° Baumé, percent by volume                                                                                                | 0.5 | 0.5  | 0.5  | 0.5 | 1.2 | 2.0 | 2.0  | 2.0 | 2.0 | 4.0 | 4.0 | 4.0  |
| (b) Alkaline Cleaning Mix:                                                                                                                                |     |      |      |     |     |     |      |     |     |     |     |      |
| Trisodium phosphate, weight percent of $\text{Na}_3\text{PO}_4 \cdot 12\text{H}_2\text{O}$                                                                | 0.5 | 4.0  | 4.0  | 0.5 | 1.8 | 0.5 | 4.0  | 2.0 | 0.5 | 2.0 | 0.5 | 4.0  |
| Milli-mol percent, any hydrate, alkaline polyphosphate, alkaline phosphate                                                                                | 1.3 | 10.5 | 10.5 | 1.3 | 4.7 | 1.3 | 10.5 | 5.3 | 1.3 | 5.3 | 1.3 | 10.5 |
| Sodium tetraborate, weight percent of $\text{Na}_3\text{B}_4\text{O}_7 \cdot 10\text{H}_2\text{O}$                                                        | 0.5 | 3.0  | 0.5  | 0.5 | 1.2 | 0.5 | 3.0  | 1.5 | 0.5 | 1.5 | 0.5 | 3.0  |
| Milli-mol percent, $\text{Na}_2\text{B}_4\text{O}_7 \cdot x\text{H}_2\text{O}$ , with $x=0$ or more                                                       | 1.3 | 7.9  | 1.3  | 1.3 | 3.2 | 1.3 | 7.9  | 1.3 | 1.3 | 3.9 | 1.3 | 3.9  |
| Sodium carbonate, weight percent of $\text{Na}_2\text{CO}_3$ , Milli-mol percent, $\text{Na}_2\text{CO}_3 \cdot x\text{H}_2\text{O}$ , with $x=0$ or more | 0.0 | 1.0  | 0.0  | 1.0 | 0.3 | 0.0 | 1.0  | 0.3 | 0.3 | 0.3 | 0.0 | 1.0  |
|                                                                                                                                                           | 0.0 | 9.4  | 0.0  | 0.4 | 2.8 | 0.0 | 9.4  | 2.8 | 2.8 | 2.8 | 0.0 | 9.4  |

Milli-mol percents in the above indicate the concentrations needed regardless of degree of hydration. The sodium silicate solution referred to has a ratio of sodium oxide to silica of not more than 1:2 not less than 1:3.5.

The respective solutions noted in the above table, (a) and (b), are separately circulated through the cooling system that is to be conditioned. The time of treatment varies widely from five minutes to four hours, and depends upon the concentration of the solution; weaker solutions require more time. The preferred embodiment is Example 5 above and the alkaline mix is circulated for about one hour.

The superiority of this new conditioning treatment lies in the fact that simultaneously with deactivation, corrosive products are sufficiently eliminated so as not to clog the cooling system on subsequent use. The chloride content is known to be indicative of the amount of soil present in the system. Fresh water has a chloride content of about 6 parts per million. Cooling systems treated with the conventional acid cleaners and flushed until the water drainings have a chloride content of 6 parts per million have after a month of use a chloride content of 200 parts per million. Studies with the present invention disclose the following results:

*Chloride contents in parts per million after at least 200 hours in dynamometer*

| Silicate Treated—Alkaline Cleaning Rinse: Trisodium phosphate, Sodium tetraborate (No Carbonate) | Silicate Treated—Alkaline Cleaning Rinse: Trisodium phosphate, Sodium tetraborate, Sodium carbonate; |
|--------------------------------------------------------------------------------------------------|------------------------------------------------------------------------------------------------------|
| 37                                                                                               | 30                                                                                                   |
| 29                                                                                               | 25                                                                                                   |
| 30                                                                                               | 16                                                                                                   |
| 6                                                                                                | 9                                                                                                    |
| -----                                                                                            | 12                                                                                                   |
| Average 32                                                                                       | 17                                                                                                   |

The maximum chloride level obtained with trisodium phosphate plus sodium tetraborate after 400 hours was 37 p.p.m. Addition of two ounces of sodium carbonate to the alkaline cleaning mix was made, primarily from a corrosion inhibition viewpoint. In the comparison study this further reduced the average to about 17 p.p.m. in 400 hours. Corresponding dynamometer studies without an alkaline rinse climbed to at least 84 p.p.m. in 400 hours. For the unused cleaned dynamometer cooling system (new) 12 p.p.m. was found. Hence, an average of 17—12=5 p.p.m. can be associated with residual soil unremoved by the alkaline cleaning treatment. Since 84—12=72 p.p.m., this is associated with residual soil without alkaline cleaning rinse,  $\frac{72}{93}$  or 7 percent remains unremoved, and the alkaline cleaning rinse is on the average 93 percent successful on this chloride criterion. This significant reduction in the chloride content in parts per million means the life of the cooling system after acid cleaning can be increased some 400 percent.

The alkali tetraborate plus the alkali phosphate form a synergistic detergent, as borate alone gives no improvement in chloride build up in vehicle studies when used for one hour at 160°—180° F. as the alkaline rinse. Then too, the average chloride content climbs to 84 p.p.m. after 200 hours operation in the dynamometer when a tri-sodium phosphate rinse is used alone, but to 32 p.p.m. when the tetraborate-phosphate mix is used for the alkaline rinse of the conditioning step. Thus, the increased detergency of the combination is readily apparent. Such increase would not be predictable from the data, as the borate alone gives no detergency effect whatsoever under these conditions and the phosphate gives a weak detergency effect.

15 In the foregoing description we have disclosed preferred embodiments of the invention. However, it is not intended that this invention be limited by specific examples set forth above and it will be apparent to those skilled in the art that variations may be made without departing from the 20 spirit of the invention as defined in the claims.

We claim:

1. A process of conditioning a cooling system after acid cleaning comprising the steps of circulating through the system an alkali metal silicate solution, draining said solution and rinsing said system with an alkaline solution containing an alkali metal phosphate and an alkali metal tetraborate.

2. The process according to claim 1 in which said alkaline rinse solution contains sodium carbonate.

30 3. The process according to claim 1 wherein the temperature range of the solutions during treatment is maintained between about 160° to 180° F.

4. The process of conditioning a cooling system after acid cleaning comprising the steps of circulating through the system an alkali metal silicate solution, draining said solution and rinsing said system with an alkaline solution comprising, by weight, of about 0.5 to 4.0 percent of an alkali metal phosphate and about 0.5 to 3.0 percent of an alkali metal tetraborate.

40 5. The process according to claim 4 in which said alkaline rinse solution contains not more than 1.0 percent by weight of sodium carbonate.

6. The process according to claim 4 in which said silicate solution is present in amounts of about 0.5 to 4.0 percent by volume.

45 7. The process according to claim 4 wherein the temperature range of the solutions during treatment is maintained between about 160° to 180° F.

8. The process of conditioning a cooling system after acid cleaning comprising the steps of circulating through the system about 0.5 to 4.0 percent by volume of a sodium silicate solution, draining said solution, and rinsing said system with an alkaline solution comprising, by weight, about 0.5 to 5.0 percent trisodium phosphate and about 55 0.5 to 3.0 percent sodium tetraborate.

9. The process according to claim 8 in which said alkaline rinse solution contains up to about 1.0 percent by weight sodium carbonate.